

# United States Patent [19]

Petersen et al.

[11] 3,920,390

[45] Nov. 18, 1975

[54] **MANUFACTURE OF FINISHING AGENTS FOR CELLULOSIC TEXTILES**

[75] Inventors: **Harro Petersen, Frankenthal; Klaus Erhardt, Leimen; Wilhelm Ruemens; Heinz Bille**, both of Limburgerhof, all of Germany

[73] Assignee: **BASF Aktiengesellschaft, Ludwigshafen (Rhine), Germany**

[22] Filed: **Sept. 26, 1973**

[21] Appl. No.: **400,720**

[30] **Foreign Application Priority Data**

Oct. 7, 1972 Germany ..... 2249320

[52] U.S. Cl. .... **8/185; 260/69 R; 117/143 A; 117/161 LN**

[51] Int. Cl.<sup>2</sup> ..... **C08G 9/10**

[58] **Field of Search** ..... **8/185; 260/69 R; 117/143 A, 161 LN**

[56] **References Cited**

UNITED STATES PATENTS

2,254,001 8/1941 Conaway ..... 8/185

|           |         |                  |       |
|-----------|---------|------------------|-------|
| 3,518,042 | 6/1970  | Pensa .....      | 8/185 |
| 3,651,139 | 3/1972  | Feinauer .....   | 8/185 |
| 3,763,106 | 10/1973 | Markiewitz ..... | 8/185 |
| 3,772,292 | 11/1973 | Martin .....     | 8/185 |
| 3,801,546 | 4/1974  | Petersen .....   | 8/185 |

## FOREIGN PATENTS OR APPLICATIONS

1,077,344 7/1967 United Kingdom

1,204,211 9/1970 United Kingdom

*Primary Examiner*—Benjamin R. Padgett

*Assistant Examiner*—D. P. Walsh

*Attorney, Agent, or Firm*—Johnston, Keil, Thompson & Shurtleff

[57] **ABSTRACT**

Process for the manufacture of liquid crease-resistant finishing agents for cellulosic textile materials, the agents being based on urea and formaldehyde, from which they are obtained by condensation in two steps at specific pH values and in specific molar ratios. The agents have a long shelf life.

**10 Claims, No Drawings**

## MANUFACTURE OF FINISHING AGENTS FOR CELLULOSIC TEXTILES

The invention relates to a process for the manufacture of crease-resist finishes for cellulosic textile materials, the agents being based on urea and formaldehyde and having a long shelf life.

For finishing cellulosic textiles, methylol compounds of cyclic ureas and, in particular, methylol compounds of urea are employed. Monomethylolurea and dimethylolurea display the greatest reactivity amongst the currently known N-methylol compounds suitable for textile finishing. They are therefore preferred. Because of their high reactivity and their limited solubility, it is not possible to prepare solutions of monomethylolurea and dimethylolurea having the shelf life required in practice. Methylolureas are crosslinked to the textile substrate in the presence of metal salt catalysts, ammonium salts or acids. If methylolureas are employed, the stability of the liquor in the presence of such catalysts is very limited.

In practice, it has for these reasons only been possible to employ the methylolureas in the form of powder grades, for example as spray-dried products. It was necessary to dissolve these solid products before use, and in the form of a solution the stability of the liquor was so limited that the products had to be used within 2 to 3 hours.

It is an object of the invention to provide aqueous solutions of finishing agents, based on urea and formaldehyde, which have a shelf life of at least three months, the liquor stability of which in the presence of catalysts is substantially improved compared to the state of the art, and which, under the conditions usually employed for finishing, display a reactivity comparable with that of methylolureas.

This object is achieved by a process for the manufacture of liquid finishing agents for cellulosic textiles, the agents having a long shelf life, wherein the reaction mixture obtainable by reaction of urea or methylolated urea or water-soluble urea-formaldehyde polycondensation products with formaldehyde in an overall molar ratio of urea: formaldehyde of 1:3 - 10 in aqueous solution at pH values between 0 and 3 is adjusted to pH values between 6 and 10 and such amounts of urea are added, at temperatures between 20° and 80°C, that an overall molar ratio of urea to formaldehyde of 1:1.5 - 2.5 results.

"Cellulosic textiles" are woven fabrics, knitted fabrics and also non-woven fabrics of which the fibers consist of natural or regenerated cellulose or which contain such fibers mixed with other fibers.

Where methylolated urea and/or urea-formaldehyde polycondensation products are employed, the "overall molar ratio" of urea to formaldehyde is to be understood as the molar ratio of urea to the sum of free formaldehyde and formaldehyde already chemically bound to urea (in the form of methylol groups or of methylene- or dimethylene-ether bridges  $-\text{CH}_2-\text{O}-\text{CH}_2-$ ).

The pH values are measured with a glass electrode.

For the first reaction, in acid solution, urea can be employed as a solid or as a solution and formaldehyde can be employed as a solution or in the form of its polymers such as, for example, paraformaldehyde, trioxane or tetroxane, or in the form of its acetals, urea being reacted with formaldehyde in the molar ratio of 1:3 to 1:10, preferably in the molar ratio of 1:4 to 1:6, in the

presence of a strong inorganic or organic acid, at pH values between 3 and 0, preferably between 1.5 and 2.5, to give precondensates containing urone. This condensation can advantageously be carried out at temperatures between 60° and 100°C, especially at 80° to 100°C.

Instead of urea it is possible to convert methylenedurea or polymethyleneurea or their methylol compounds, such as, for example, urea-formaldehyde polycondensates, into precondensates containing urone by means of formaldehyde. It is also possible to use, as starting materials for the manufacture of the precondensates containing urone, the mixtures which result from the methylolation of urea with formaldehyde and which contain, in addition to free formaldehyde, inter alia the methylol compounds of urea, that is to say monomethylolurea, dimethylolurea, trimethylolurea and/or tetramethylolurea.

Suitable acid catalysts are inorganic acids, such as hydrochloric acid, sulfuric acid and phosphoric acid, and strong organic acids such as o-toluenesulfonic acid, oxalic acid and phthalic acid.

The reaction of the first stage can be carried out by treating the mixture of the abovementioned starting substances and formaldehyde with an acid and then heating it to the desired condensation temperature. It is however also possible first to heat the mixture of the starting substances with formaldehyde or its derivatives to the condensation temperature and only then to add the acid. According to a preferred embodiment, formaldehyde is mixed with the acid and heated to the desired condensation temperature. Urea or the abovementioned starting products are then introduced into this solution. In all embodiments it is also possible to employ mixtures of the starting components. The reaction time depends on the temperature, amount and strength of acid, and molar ratio and concentration of the starting substances.

In the acid condensation of 1 mole of urea with more than 3 moles of formaldehyde at a pH below 3, a partial cyclo-condensation to methylolated urones of the general formula



wherein  $n = 1, 2$  or  $3$ , was found to take place. The formation of the urones can be followed by means of Raman spectroscopy; they show a strong emission line in the Raman spectrum at  $810 \text{ cm}^{-1}$ . The urone content can be determined quantitatively by measuring the intensity of the line.

A factor of great importance to the shelf life of the products claimed according to the invention is that the acid condensation of urea with formaldehyde to give products containing urone is carried out in such a way that certain limiting conditions are observed. Thus, in particular when using molar ratios of about 1:3 to 4 in the 1st stage of the reaction, it is necessary to ensure that the neutralized samples do not become turbid or precipitate after standing for a short time. Such turbidity can occur regardless of the amount of acid chosen.

On lowering the molar ratio of urea to formaldehyde, the values at which turbidity is found shift to a higher degree of cyclization. Thus, for example, in the condensation of urea with formaldehyde in a molar ratio of 1:4 at a temperature of 100°C in the presence of 1 to 5 ml of 75 percent strength sulfuric acid per kg of reaction mixture the degree of cyclization at which turbidity is found is approx. 45 percent, whilst for a molar ratio of 1:6 and under otherwise identical conditions this value is about 55 to 60 percent.

According to the present invention, the intermediates containing urone and free formaldehyde can be converted by further reaction with urea into aqueous finishing agents which display high reactivity, high stability and, in contrast to the aqueous solutions of the methylolureas, excellent liquor stability. For this purpose, the precondensates obtained in the manner described are reacted with such amounts of urea as to give an overall molar ratio of urea to formaldehyde of 1:1.5 - 2.5, preferably of 1:1.7 - 2.3. The urea can be added in the form of a solid or as a solution. The reaction takes place at a pH between 6 and 10, preferably between 6.4 and 9 and at temperatures between 20° and 80°C, preferably at 30° to 60°C. The reaction time depends on the temperature and on the pH and is between one and five hours. The reaction can be followed, for example, by continuous quantitative determination of the free formaldehyde in the solution. The reaction is complete when the concentration of free formaldehyde shows practically no further decrease.

The liquid textile finishes thus produced show an excellent shelf life. When stored at temperatures below 25°C, they remain usable for at least 6 months. This was not foreseeable.

The new finishing agents are employed in conventional manner, preferably in the form of an aqueous impregnating bath to which the catalysts generally required for the crosslinking reaction are added. Potentially acid catalysts, which are generally known, and customary, for textile finishing purposes, are particularly suitable. Examples of catalysts of this type which can be used are ammonium salts of strong acids, magnesium chloride, zinc chloride and zinc nitrate. Mixtures of several catalysts can also be used. The concentration of finishing agent depends, in the usual way, on the desired effect and is generally between 50 and 200 g/l. The goods being treated are impregnated with the impregnating liquor in the usual way. Preferably, a padder is used for this purpose. The impregnated goods are freed from excess impregnating liquid in a known manner, for example by squeezing out. It is possible to dry the impregnated fibrous goods to a greater or lesser extent and then heat them to a temperature of 100 to 210°C, preferably 130° to 180°C, in the presence of the acid or potentially acid catalysts. In general, fixing is complete after 1 to 6 minutes under these conditions. It is possible mechanically to shape the fibrous goods during or after drying before fixing, for example by compression, crimping, ironing, calendering, embossing or pleating. Cellulosic textiles are given a durable crease-resist and shrink-resist finish in this way and the embossed effects and pleats are relatively resistant to laundering.

The previously used hydroxymethyl or alkoxyethyl compounds containing nitrogen, as well as finishing agents not containing nitrogen, can be used conjointly with the new agents. It is also possible to use, conjointly, the customary water repellents, softeners, leveling

agents, wetting agents, etc., such as, in particular, polymer solutions or dispersions. Examples of water repellents are paraffin wax emulsions containing aluminum or zirconium, preparations containing silicones, and perfluorinated aliphatic compounds. Softeners which may be mentioned are oxyethylation products of higher fatty acids, fatty alcohols or fatty acid amines, higher-molecular polyglycol ethers, higher fatty acids, fatty alcohol sulfonates, N-stearyl-N', N'-ethylideneurea and stearylaminomethylpyridinium chloride. Examples of levelling agents which can be used are water-soluble salts of acid esters of polybasic acids with ethylene oxide adducts or propylene oxide adducts of long-chain basic starting material which can be oxyalkylated. Examples of wetting agents are salts of alkylnaphthalene-sulfonic acids, the alkali metal salts of sulfonated succinic acid diethyl ester and the adducts of alkylene oxides to fatty alcohols, alkylphenols, fatty amines and the like. Examples of finishes which can be used are cellulose ethers or cellulose esters and alginates, and also solutions or dispersions of synthetic polymers and polycondensates, for example of polyethylene, polyamides, oxyethylated polyamides, polyvinyl ethers, polyvinyl alcohols, polyacrylic acid or its esters and amides and corresponding polymethacrylic compounds, polyvinylpropionate, polyvinylpyrrolidone and copolymers, for example those of vinyl chloride and acrylates, of butadiene and styrene or acrylonitrile or of vinylidene chloride,  $\beta$ -chloroalkylacrylates or vinyl ethyl ether and acrylamide or the amides of crotonic acid or maleic acid, or of N-methylolmethacrylamide and other polymerizable compounds. These additional auxiliaries are in general employed in amounts of 0.3 to 4 percent, preferably 1 to 2.5 percent, relative to the weight of the dry textile goods; in special cases, these amounts can be exceeded.

The parts and percentages mentioned in the Examples which follow are units by weight. The relationship of parts by weight to parts by volume is as that of one kilogram to one liter.

#### EXAMPLE 1

2 parts of 50 percent strength sulfuric acid are added to 540 parts of a 40 percent strength formaldehyde solution and the mixture is heated to 90°C. 157.8 parts of a 68.5% strength urea solution are introduced at this temperature over a period of 30 minutes. The pH is 1 to 1.1. The reaction mixture is heated at 90°C for 30 minutes and is then cooled to 45°C, and its pH is adjusted to pH 6.8 with approx. 1.2 parts of 50 percent strength sodium hydroxide solution. This solution contains approx. 33 percent of the urea in the form of urones. 157.8 parts of a 68.5 percent strength urea solution are introduced into this mixture, whilst stirring. The reaction solution is heated at 50°C for 4 hours whilst maintaining a pH of 6.8 to 7.0. Approx. 840 parts of the finishing agent, with a solids content of 48 percent, are obtained. The free formaldehyde content is 0.8 percent.

#### EXAMPLE 2

1,350 parts of a 40 percent strength formaldehyde solution and 263 parts of a 68.5 percent strength urea solution are heated to 100°C in a stirred flask. After adding 4.5 parts of 75 percent strength sulfuric acid, the mixture is stirred for 90 minutes at 100°C. The reaction solution is then adjusted to pH 7.0-7.2 with 50 percent strength sodium hydroxide solution whilst at

the same time cooling it to 45°C. This solution contains approx. 54 percent of the urea in the form of urone. 526 parts of a 68.5 percent strength urea solution are added at 45°C. The reaction mixture is stirred for 4 hours at 50°C whilst keeping the pH at 7.2-7.4 by adding triethanolamine. 2,150 parts of a 48 percent strength solution of the finishing agent according to the invention, containing 2.1 percent of free formaldehyde, are obtained.

## EXAMPLE 3

1,440 parts of a 60 percent strength methylolatior mixture of urea with formaldehyde, in the molar ratio of 1:4, are heated to 100°C and stirred with 4 parts by volume of 75 percent strength sulfuric acid for 10 minutes at 100°C. The reaction mixture is then immedi-

## EXAMPLE 5

A bleached and mercerized cotton fabric (120 g/m<sup>2</sup>) is padded with a finishing liquor which contains 120 parts of the product prepared according to Example 1 and 3 parts of ammonium chloride per liter. The wet pickup is 70 percent. The fabric is dried out and then the condensation reaction is carried out for 4 minutes at 140°C (the test results are given in column A of the table). A comparison experiment is carried out with a fresh solution of 70 parts of crystalline dimethylolurea and 4 parts of ammonium chloride, dissolved in 1 liter of water (column C). After 6 hours, the solutions are again applied to untreated fabric of the type described above (columns B and D). At this stage, the solution of the crystalline dimethylolurea is already very turbid.

| RESULTS:                                 | Product accord- |           | Dimethylol- | Untreated |
|------------------------------------------|-----------------|-----------|-------------|-----------|
|                                          | according to    | Example 1 | urea        | fabric    |
|                                          | A               | B         | C           | D         |
| Dry crease angle according to DIN 53,890 |                 |           |             |           |
| Sum of warp + weft                       | 220             | 218       | 205         | 210       |
| After 1 machine wash at 60°C             | 208             | 205       | 180         | 152       |
| Decrease in tensile strength in %        | 25              | 26        | 30          | 29        |
|                                          |                 |           |             | 0         |

ately adjusted to pH 7 with a 50 percent strength sodium hydroxide solution, whilst cooling. At this stage, the mixture contains approx. 40 percent of the urea in the form of urone. 288 parts of crystalline urea are added to this precondensate containing urone. The mixture is stirred for 3 hours at 45 to 50°C whilst maintaining a pH of 7.2-7.4, the pH being adjusted with triethanolamine or dimethylethanolamine. 1,740 parts of an approx. 60 percent strength finishing agent, containing approx. 1.5 percent of free formaldehyde, are obtained.

30

## EXAMPLE 6

Unbleached rayon staple cloth (140 g/m<sup>2</sup>) is padded with a finishing liquor which contains, per liter, 200 parts of the product prepared according to Example 2 and 30 parts of a 30 percent strength zinc nitrate solution. The wet pickup is 90 percent. After drying the fabric, the condensation reaction is carried out for 4 minutes at 140°C. A comparison experiment is carried out with a freshly prepared liquor of 110 parts of dimethylolurea and 30 parts of a 30 percent strength zinc nitrate solution per liter.

| RESULTS:                                 | Product accord- |           | Dimethylol- | Untreated |
|------------------------------------------|-----------------|-----------|-------------|-----------|
|                                          | according to    | Example 2 | urea        | fabric    |
|                                          | A               | B         | C           | D         |
| Dry crease angle according to DIN 53,890 |                 |           |             |           |
| Warp + weft                              | 215             | 210       | 188         | 95        |
| After 1 wash at 60°C                     | 200             | 188       |             | 90        |
| Monsanto rating* after one wash at 60°C  | 4.75            | 4.25      |             | 1.25      |

\*Compare AATCC Technical Manual 88A-1964 T.

## EXAMPLE 4

1,000 parts of a 65 percent strength polycondensation product of urea with formaldehyde in the molar ratio of 1:1.6 are mixed with 2,140 parts of 40 percent strength formaldehyde solution and the mixture is heated to 90°C. After adding 7 parts by volume of 75 percent strength sulfuric acid, the mixture is stirred at 90°C for 1½ hours, and is then neutralized with dilute sodium hydroxide solution, whilst cooling it. At 50°C, 780 parts of crystalline urea are added to the reaction mixture. The reaction solution is heated at 50°C for three hours whilst maintaining a pH of 7.2-7.6 by means of triethanolamine. 3,950 parts of an approx. 55 percent strength aqueous solution are obtained.

55 An embossed effect produced on a ribbed calendar prior to the condensation reaction shows similar durability to laundering in both products.

We claim:

1. A process for the manufacture of a liquid finishing agent for cellulosic textiles which is stable on storage, wherein a reaction mixture obtainable by reaction of urea or methylolated urea or a water-soluble urea-formaldehyde polycondensation product with formaldehyde in an overall molar ratio of urea: formaldehyde of from 1:3 to 1:10 in aqueous solution at a pH of from 0 to 3 is adjusted to a pH of from 6 to 10 and urea is added at a temperature of from 20° to 80°C to provide an overall molar ratio of urea to formaldehyde of from 1:1.5 to 1:2.5.

2. A process as claimed in claim 1 wherein the reaction mixture is obtained by reaction of urea or methylolated urea or a water-soluble urea-formaldehyde condensation product with formaldehyde in an overall molar ratio of urea: formaldehyde of from 1:4 to 1:6 in aqueous solution at a pH of from 0 to 3.

3. A process as claimed in claim 2 wherein the reaction mixture is obtained at a pH of from 1.5 to 2.5.

4. A process as claimed in claim 2 wherein the formaldehyde for reaction with the urea, methylolated urea or water-soluble urea-formaldehyde condensation product is provided in the form of a polymer or acetal thereof.

5. A process as claimed in claim 2 wherein the reaction of urea, methylolated urea or water-soluble urea-formaldehyde condensation product with formaldehyde is carried out in the presence of a mineral acid or

strong organic acid at a temperature of from 60° to 100°C.

6. A process as claimed in claim 1 wherein the pH of the initial reaction mixture is adjusted to from 6.4 to 9 and urea is added to provide an overall molar ratio of urea to formaldehyde of from 1:1.7 to 1:2.3.

7. Liquid finishing agents for cellulosic textiles when manufactured by the process of claim 1.

8. A process for finishing cellulosic textiles wherein the textile material is treated with a liquid finishing agent as claimed in claim 7.

9. A process as claimed in claim 8 wherein the textile material is treated in an aqueous impregnating bath containing the liquid finishing agent and a potentially acid crosslinking catalyst.

10. Cellulosic textiles which have been finished by a process as set forth in claim 8.

\* \* \* \* \*